

# UNITED STATES PATENT OFFICE.

AXEL FRANCK-PHILIPSON, OF CHICAGO, ILLINOIS.

## PROCESS FOR REMOVING NATURAL ENAMEL FROM THE SURFACE OF RATAN, &c.

1,296,553.

Specification of Letters Patent.

Patented Mar. 4, 1919.

No Drawing. Application filed May 31, 1916, Serial No. 100,923. Renewed January 25, 1919. Serial No. 273,169.

*To all whom it may concern:*

Be it known that I, AXEL FRANCK-PHILIPSON, subject of the King of Denmark, residing at Chicago, in the county of Cook 5 and State of Illinois, have invented certain new and useful Improvements in Processes for Removing Natural Enamel from the Surface of Ratan, Bamboo, and the like; and I do hereby declare the following to 10 be a full, clear, and exact description of the invention, such as will enable others skilled in the art to which it appertains to make and use the same.

This invention has for its object to pro-

15 vide a novel process for removing the natural gloss, enamel or shell coating from bamboo or ratan, and consists in the several steps hereinafter fully described and claimed.

20 Heretofore, as far as I am informed, this gloss, enamel or shell has been mechanically removed from the ratan or bamboo at considerable expense, and that all attempts to chemically remove the same have proved 25 unavailing.

The object of my present invention is, therefore, to provide a process for chemically removing this gloss from ratan at a cost less than the mechanical removal 30 thereof, and in such a manner as not to injure the fiber of the ratan subjected to the process, and so that it will lend itself readily to bleaching by the process described in Letters Patent No. 1,068,580 granted to me 35 or by any other suited to the purpose.

My said invention consists broadly in subjecting the ratan to the action of a solvent for the said gloss or shell, and I have found that this can be accomplished in several 40 ways.

In its preferred form my said method consists in subjecting the ratan to the action of a relatively strong solution of alkaline hydrate, preferably caustic soda. A satisfactory solution well adapted for the purpose consists of one hundred pounds, more or less, of caustic soda, and twelve hundred gallons, more or less, of water.

45 Preferably the treatment consists in immersing the ratan in this solution in the presence of heat for a period of one-half an hour to two hours, more or less, the length of time varying with the strength of the solution, and the temperature of the latter. I 50 have found that if the solution is main-

tained at the boiling point it will remove the gloss from the ratan or reed in the shortest time, the duration depending upon the particular kind of ratan treated.

While the foregoing solution effectually 60 removes the gloss or natural enamel from the ratan I have found that it has the effect of roughening the surface somewhat and that better results are obtained by adding to the bath aforesaid, five gallons, more or less, 65 silicate of soda, the result being that the ratan is left smoother and in better condition than if the said silicate of soda is omitted.

Other alkaline hydrates may be substituted, as for example, potassium hydrate, calcium hydrate, and the like, the sodium hydrate being, however, preferable and giving the most satisfactory results.

As the ratan leaves the solution it will be 75 found to be black, or of a very dark color, but this is merely on the surface and may be removed by subjecting the ratan to the action of any suitable bleaching process, such for example as is described in Letters 80 Patent No. 1,068,580 granted to me on August 12, 1913, being preferable. The usual chlorinated lime or chlorin gas bleaching process may also be used, but this is apt to deleteriously affect the fiber of the ratan. 85

I have found that ratan grown in different localities differs quite materially in the character of the surface gloss or enamel which it is desired to remove preparatory to using such ratan in the manufacture of furniture and the like. I have found, for example, that ratan grown in one locality has a comparatively thin shell coating of silicate; whereas in other localities this coating is very much thicker, and in all instances 90 it is probable that the silicate is mixed more or less with a resinous sap. The differences in the various qualities affect the time required for the removal of this enamel or gloss so that the process must be varied 100 as to its duration in accordance with the particular character of the ratan treated.

I claim as my invention:

1. The herein-described process for removing the natural enamel from the surface of 105 ratan and the like which consists in subjecting said material to the action of an alkaline hydrate solution containing silicate of soda.

2. The herein-described process for removing the natural enamel from the surface of 110

ratan and the like which consists in subjecting said material to the action of a hot alkaline hydrate solution containing silicate of soda.

5. 3. The hereindescribed process for removing the natural enamel from the surface of ratan and the like which consists in subjecting said material to the action of a boiling alkaline hydrate solution containing silicate of soda.

10. 4. The hereindescribed process for removing the natural enamel from the surface of ratan and the like which consists in subjecting said material to the action of an alkaline hydrate solution containing silicate of soda for a period varying from one-half hour to two hours, more or less.

15. 5. The hereindescribed process for removing the natural enamel from the surface of

ratan and the like which consists in subjecting said material to the action of a hot alkaline hydrate solution containing silicate of soda for a period varying from one-half hour to two hours, more or less.

20. 6. The hereindescribed process for removing the natural enamel from the surface of ratan and the like which consists in subjecting said material to the action of a boiling alkaline hydrate solution containing silicate of soda for a period varying from one-half hour to two hours, more or less.

25. In testimony whereof I have signed my name in presence of two subscribing witnesses.

AXEL FRANCK-PHILIPSON.

Witnesses:

M. M. BOYLE,  
G. M. WALKER, Jr.

Copies of this patent may be obtained for five cents each, by addressing the "Commissioner of Patents,  
Washington, D. C."